

## 1

3,485,624

PHOTOCONDUCTIVE PROPERTIES OF  
POLY-N-VINYL CARBAZOLE

Roger P. J. G. Thiebaut, Jean-Pierre C. G. Dubosc, and  
Claude A. L. L. Mercier, Vincennes, France, assignors  
to Eastman Kodak Company, Rochester, N.Y., a cor-  
poration of New Jersey  
No Drawing. Filed June 7, 1966, Ser. No. 555,664  
Int. Cl. G03g 5/06; C08f 7/16  
U.S. Cl. 96—1.5

2 Claims

## ABSTRACT OF THE DISCLOSURE

According to the present invention, a substantial increase in photographic speed of photoconductive coatings containing poly-N-vinyl carbazole is obtained by heat treatment of such coatings at a temperature in the range from about 250° C. to about 300° C. for a time period from about 15 minutes to about 1 hour.

This invention relates to electrophotography. More particularly, the invention relates to electrophotographic elements comprising a photoconductive insulating coating on a support.

Poly-N-vinyl carbazole is a compound used for its photoconductive properties in certain reproduction processes which utilize electrostatic charges. Use of poly-N-vinyl carbazole as an organic photoconductor in electrophotographic elements is described in numerous literature references, for example, in U.S. Patent No. 3,037,861, patented June 5, 1962.

An object of the invention is to provide improved electrophotographic elements comprising an annealed photoconductive coating containing the organic photoconductor, poly-N-vinyl carbazole.

Another object of the invention is to provide a method for improving the photographic speed of photoconductive electrically insulating coatings containing the organic photoconductor, poly-N-vinyl carbazole.

According to the present invention, a substantial increase in photographic speed of photoconductive coatings containing poly-N-vinyl carbazole is obtained by heat treatment of such coatings at a temperature in the range from about 250° C. to about 300° C. for a time in the range from about 15 minutes to about 1 hour. The higher the temperature, the shorter the time. At temperatures lower than 250° C., the effect is negligible, whereas at temperatures above 300° C. the degradation of the polymer is too important for it to be used in a photoconductive coating.

## 2

It has also been found that much more sensitive photoconductive coatings were obtained when crystalline poly-N-vinyl carbazole was used instead of the amorphous polymer. By comparison with the amorphous poly-N-vinyl carbazole, the crystalline polymer shows a  $T_{1/10}$  period, such as defined hereunder, which is more than twice smaller (about 6 to 8 seconds instead of 17 to 20 seconds) and the practical exposure time, which is also defined hereunder, is divided by a still greater factor (4 to 5 seconds instead of 12 to 30 seconds).

In this specification, the  $T_{1/10}$  period is the time required for the potential of a photoconductive layer to reach  $\frac{1}{10}$  of the value of the potential after the initial charge, when said layer is subjected to an illumination of 13,600 lx. The practical exposure time is the minimum exposure time in seconds, under the same 13,600 lx. illumination, required to obtain the best possible image without any background fog, with magnetic brush development. Thus the lowest number indicates the highest photographic speed.

The heat treatment may be conducted as well on coatings comprising either commercial amorphous poly-N-vinyl carbazole or on crystalline poly-N-vinyl carbazole. Examples of commercial amorphous poly-N-vinyl carbazole are Luvican M-170 or M-710 sold by Badische Anilin Soda Fabrik. Crystalline polymers with which we experimented were synthesized in our laboratory by the process described in Belgian Patent No. 606,790. With both amorphous and crystalline samples, the results obtained by heat treatment were quite similar. We prefer the crystalline materials because they provide better resistance to degradation by heating. With both types, however, at the annealing temperatures used, heat degradation was slight enough to be tolerable.

The following examples are provided to describe certain preferred embodiments of the invention.

## EXAMPLE 1

A solution of poly-N-vinyl carbazole in benzene is prepared by dissolving 6 gm. Luvican M-170 in 100 ml. benzene. The solution is coated on an aluminum plate and the solvent is evaporated at room temperature in air, leaving a film of poly-N-vinyl carbazole coated on the metal support. The coating is electrically insulating and photoconductive. The coated plate is placed in an electric oven in a nitrogen atmosphere and heated to annealing temperature; the sample is annealed for a period in the range from about 15 minutes to about 1 hour. In Table 1 are tabulated descriptions of test results obtained with samples prepared as described above and annealed for the times and at the temperatures shown in the table.

TABLE 1

| Heat treatment   | Coating thickness in microns | Initial potential (volts) | Reduction of charge in darkness, 3 minutes (percent reduction) | $T_{1/10}$ | Practical exposure time (seconds) |
|------------------|------------------------------|---------------------------|----------------------------------------------------------------|------------|-----------------------------------|
| None             | 10                           | 800                       | 10                                                             | 1.7        | 30                                |
| 15 min., 250° C. | 10                           | 1,000                     | 33                                                             | 1.7        | 2                                 |
| 60 min., 250° C. | 8                            | 650                       | 30                                                             | 1.4        | 2                                 |
| 15 min., 275° C. | 8                            | 600                       | 19                                                             | 3.7        | 5                                 |
| 60 min., 275° C. | 6                            | 490                       | 28                                                             | 1.1        | 1.4                               |
| 15 min., 300° C. | 9                            | 800                       | 24                                                             | 1.4        | 1.4                               |

The test results tabulated in Table 1 were obtained by first dark-adapting each plate for several days and then applying an electrostatic charge by means of corona discharge. The natural charge decay after 3 minutes was observed and recorded. The  $T_{1/10}$  period and the practical exposure time, such as defined above, were also observed and recorded.

#### EXAMPLE 2

The procedure of Example 1 was repeated, except that the coating solvent used was a 53/33/14 mixture of benzene, methylene chloride and dioxane, with poly-N-vinyl carbazole prepared by the process described in the aforesaid Belgian Patent No. 606,790. In Table 2 are tabulated tests results obtained as in Example 1.

TABLE 2

| Heat treatment        | Coating thickness in microns | Initial potential (volts) | Reduction of charge in darkness, 3 minutes (percent reduction) | $T_{1/10}$ | Practical exposure time (seconds) |
|-----------------------|------------------------------|---------------------------|----------------------------------------------------------------|------------|-----------------------------------|
| None-----             | 13                           | 1,200                     | 12                                                             | 6-8        | 4                                 |
| 60 min., 250° C-----  | 10                           | 1,200                     | 40                                                             | 0.4        | —                                 |
| 180 min., 250° C----- | 10                           | 1,000                     | 74                                                             | 0.1        | —                                 |
| 480 min., 250° C----- | 8                            | 1,200                     | 43                                                             | 0.1        | —                                 |
| 180 min., 275° C----- | 10                           | 550                       | 78                                                             | 0.3        | —                                 |
| 180 min., 275° C----- | 10                           | 950                       | 85                                                             | 0.2        | —                                 |
| 180 min., 300° C----- | 13                           | 1,000                     | 61                                                             | 0.4        | —                                 |
| 60 min., 330° C-----  | 12                           | 210                       | 65                                                             | 3.5        | —                                 |

In the last column of Table 2, the sign (—) indicates that the practical exposure time is too small to be measured.

In describing certain preferred embodiments of our invention, we have used coatings consisting essentially of poly-N-vinyl carbazole. However, our invention extends to use of the improvements with poly-N-vinyl carbazole in electrophotographic photoconductive coatings which may also contain other organic polymers in combination with poly-N-vinyl carbazole. Such coatings are described in the literature. Our invention further extends to use of the improvements with photoconductive coatings containing photoconductive poly-N-vinyl carbazole with added sensitizers, activators, and the like, of various kinds known and used in the arts relating to organic photoconductive coatings.

It will be understood that modifications and variations

may be made within the scope of the invention as described above and as defined in the following claims.

We claim:

1. A method for improving the photographic speed of electrophotographic elements comprising a support and coated thereon a photoconductive electrically insulating layer comprising photoconductive poly-N-vinyl carbazole, said method comprising the step of annealing said electrophotographic element at a temperature in the range from 250-300° C. for a time in the range from 15 minutes to 1 hour.

2. An improved electrophotographic element for use in electrophotography comprising a support and coated thereon an annealed, electrically insulating photoconduc-

tive coating comprising photoconductive poly-N-vinyl carbazole, said element having been heat-annealed at a temperature in the range from 250-300° C. for a time in the range from about 15 minutes to about 1 hour.

#### References Cited

##### UNITED STATES PATENTS

2,863,767 12/1958 Vyverberg et al. ----- 96—1  
3,037,861 6/1962 Hoegl et al. ----- 96—1.5  
3,421,891 1/1969 Inami et al. ----- 96—1.6

40 GEORGE F. LESMES, Primary Examiner

C. E. VAN HORN, Assistant Examiner

U.S. CL. X.R.

45 252—501; 260—88.3